

## United States Patent [19]

Croon et al.

[11] 3,802,958

[45] Apr. 9, 1974

## [54] CHLORINATION OF CELLULOSE PULP

[75] Inventors: Ingemar Liss-Albin Croon,  
Salvgagen; Sten Oskar Dillén,  
Strandvagen, both of Sweden

[73] Assignee: Mo och Domsjo Aktiebolag,  
Ornsköldsvik, Sweden

[22] Filed: Apr. 8, 1971

[21] Appl. No.: 132,367

## Related U.S. Application Data

[63] Continuation-in-part of Ser. No. 774,171, Nov. 7,  
1968, abandoned.

[52] U.S. Cl. .... 162/89, 8/108

[51] Int. Cl. .... D21c 9/12

[58] Field of Search ..... 162/89, 88, 87; 8/108

## [56] References Cited

## UNITED STATES PATENTS

|           |         |                  |          |
|-----------|---------|------------------|----------|
| 3,560,330 | 2/1971  | Ahlborg .....    | 162/89 X |
| 3,433,702 | 3/1969  | Jack et al.....  | 162/88 X |
| 3,652,388 | 3/1972  | Croon et al..... | 162/89 X |
| 3,536,577 | 10/1970 | Rapson .....     | 162/89 X |
| 2,166,330 | 7/1939  | Vincent .....    | 162/87 X |

## OTHER PUBLICATIONS

Rydholm, Pulping Processes, 1965, p. 839.  
Scott Paper Company Handbook, 1st ed., 1956, p. 95.

Primary Examiner—S. Leon Bashore  
Assistant Examiner—Arthur L. Corbin

## [57] ABSTRACT

A process is provided for delignifying cellulose pulps that have previously been subjected to treatments with chlorine, or chlorine dioxide, or a mixture thereof, and with alkali, and is intended to be carried out as a third or subsequent stage in the multi-stage bleaching of cellulose pulp, which comprises delignifying the cellulose pulp with a mixture of chlorine and chlorine dioxide comprising from about 10 to about 50 percent chlorine dioxide calculated as available chlorine, at a pH within the range from about 1 to about 3.5 and at a pulp consistency within the range from about 3 to about 15 percent, and a temperature within the range from about 40° to about 70° C., for a time within the range from about 30 to about 300 minutes.

7 Claims, No Drawings

## CHLORINATION OF CELLULOSE PULP

This application is a continuation-in-part of Ser. No. 774,171, filed Nov. 7, 1968, and now abandoned.

This invention relates to a process for delignifying cellulose pulp that has previously been subjected to treatments with chlorine, or chlorine dioxide, or a mixture thereof, and then with alkali; and more particularly, to a multi-stage process for bleaching cellulose pulp which includes as a third or later treatment stage, following treatment with chlorine, or chlorine dioxide, or mixture thereof, and with alkali, a delignification stage with a mixture of chlorine and chlorine dioxide at a temperature within the range from about 40° to about 70° C. for a time within the range from about 30 to about 200 minutes, and at a pulp consistency within the range from about 3 percent to about 15 percent.

The bleaching of cellulose pulp obtained by either the sulfate or sulfite process is a multi-stage procedure, and usually includes as separate steps in any of a larger number of sequences of one or more of each,

- a. a chlorination stage,
- b. an alkali treatment or alkali extraction stage,
- c. a hypochlorite treatment stage, and
- d. a chlorine dioxide treatment stage.

These treatments can be carried out in almost any order, and two or more of such stages are frequently included, but usually not in succession, but interleaved with one or more of the other stages.

In general, sulfate pulps require more treatment stages for complete bleaching than sulfite pulps. Also, in the case of sulfate pulps, chlorination, alkali treatment and chlorine dioxide treatment are almost always necessary while the hypochlorite treatment can sometimes be omitted, whereas in the case of sulfite pulps, either the hypochlorite or the chlorine dioxide treatments can be omitted, and the bleaching can be reduced to as little as three or four stages. However, all multi-stage bleaching processes employ a chlorination stage and an alkali treatment stage, and the reason is that these stages are required for delignification. Some sulfate pulps are more difficult to delignify than others, and in the case of these pulps, one chlorination stage may be insufficient to delignify the pulp sufficiently. Hence, a complementary delignification stage can be carried out in an additional chlorination stage, or in a hypochlorite treatment stage, or in a chlorine dioxide treatment stage.

The conditions under which the various treatment stages are carried out in conventional bleaching processes are summarized in Table A, which follows:

Chlorine is considered to be the most effective and least expensive of the delignifying agents that are available. However, it has a tendency to decompose the cellulose, and therefore it is necessary to keep the amount of chlorine at the minimum that will give effective delignification. The chlorination thus is usually carried out in such a manner that there is a small excess of chlorine present at the conclusion of the chlorination. This excess is rather important to control. If there is too high an excess remaining, then the tendency of the chlorination stage to decompose cellulose is increased, and if there is no excess, or if the excess is too small, the delignification of the cellulose is incomplete. If the chlorination must be applied in two stages, the risk of decomposition of the cellulose is increased in the second stage, and therefore the arrangement of the treatment stages is usually such that the chlorination is restricted to one stage, and a substitute hypochlorite or chlorine dioxide stage is used instead, if possible.

10 The chlorination, stage C, is normally performed with a relatively low pulp consistency, from about 1 to about 4 percent, and at low temperatures, from about 5° to about 25° C., for short treatment times, from about 1/3 to about 2 hours. The quantity of chlorine used varies with the properties of the unbleached pulp, but is sufficient only to give an excess within the range from about 0.1 to about 0.5 percent chlorine, based on the weight of the dry pulp, at the conclusion of the treatment.

15 Chlorine dioxide can also be used in place of chlorine in the chlorination stage. In this event, the amount of chlorine dioxide used is sufficient to supply an amount of chlorine within the range set out above sufficient to ensure an excess of from 0.1 to 0.5 percent chlorine at the end of the treatment.

20 The alkali extraction, stage E, is designed to remove the lignins that have been made alkali-soluble in the chlorination stage, and is carried out at a relatively high pulp consistency. This is normally at from about 4 percent to about 18 percent; when using presses for dewatering, up to 30 percent. The temperature can be rather low, from 25° to 30° C., but in the so-called hot alkali refining processes, for producing pulp with a high alpha cellulose content, temperatures of up to 130° C. can be employed. The treatment time can be very short, for just several minutes, up to from 4 to 5 hours. The amount of alkali charged to the system varies according to the properties of the pulp which it is desired to produce. In the case of paper pulps, it is usually carried out in such a manner that the pH at the conclusion of the

25

30

35

40

45

50

TABLE A

| Stage  | Treatment                                                            | Pulp consistency, percent | Temperature (° C.) | Time                          | Amount                                                                                                                                                                                                             |
|--------|----------------------------------------------------------------------|---------------------------|--------------------|-------------------------------|--------------------------------------------------------------------------------------------------------------------------------------------------------------------------------------------------------------------|
| C..... | Chlorination (Cl <sub>2</sub> or ClO <sub>2</sub> , or both).        | 1-4                       | 5-25               | 1/2-2 hours.....              | Enough Cl <sub>2</sub> or ClO <sub>2</sub> to provide an end of treatment 0.1 to 0.5% excess Cl <sub>2</sub> based on pulp weight.                                                                                 |
| E..... | Alkali extraction (NaOH).                                            | 4-18                      | *25-80             | Several minutes to 4-5 hours. | Enough NaOH to give a pH 8-12.5 at end of treatment.                                                                                                                                                               |
| H..... | Hypochlorite (Na OCl) or Ca (OCl) <sub>2</sub> excess alkali (NaOH). | 4-18                      | 25-60              | 1-4 hours.....                | From 0.2 to 3% Cl <sub>2</sub> to provide at end of treatment a 0.1% Cl <sub>2</sub> excess, based on pulp weight, and alkali (normally between 10 and 100% of chlorine amount) to give a pH > 8.5, usually 10-11. |
| D..... | Chlorine dioxide (ClO <sub>2</sub> ).                                | 4-15                      | 50-90              | 2-5 hours.....                | Enough to provide 0.5 to 5% Cl <sub>2</sub> , based on pulp weight, with an excess of from 0.1 to 0.5% Cl <sub>2</sub> at end of treatment.                                                                        |

\*Up to 130° C. in hot alkali refining.

treatment is within the range from about 8 to about 12.5, generally about 11.

The hypochlorite treatment, stage H, is also carried out at relatively high pulp consistencies, normally from about 4 percent to about 18 percent. The temperatures are usually rather higher than in the chlorination, and range from about 25° to about 60° C. The treatment time is also somewhat longer, from 1 hour and upwards, normally from two to four hours. The quantity of hypochlorite charged to the system varies with the type of pulp and the conditions, and is based on the amount of chlorine provided. The amount can range from very small amounts, of the order of 0.2 percent Cl<sub>2</sub> by weight of the pulp, to 3% Cl<sub>2</sub>, based on the weight of dry pulp. This treatment is also carried out in a manner to ensure that a small excess of chlorine remains at the conclusion of the treatment, about 0.1 percent by weight of the pulp.

Hypochlorite having a pH at about and immediately below the neutral point of 7 strongly decomposes cellulose, and consequently an amount of alkali is also charged to the system to provide a surplus of alkali, and maintain the pH well above 7. The amount of alkali charged as NaOH can be within the range from about 10 percent to about 100 percent by weight of the chlorine charged to the system in this stage, so as to ensure that at the conclusion of the hypochlorite treatment the pH is above 8.5, and is normally within the range from 10 to 11.

The chlorine dioxide treatment is carried out with the same pulp consistency as the hypochlorite treatment, although in practice a somewhat lower consistency can be used, since the chlorine dioxide is obtained in a more dilute form than the hypochlorite solution. Thus, the pulp consistency during chlorine dioxide treatment can be within the range from about 4 percent to about 15 percent. The temperature is higher, within the range from about 50° to about 90° C., and normally about 70° C. The treatment time is at least 2 hours, and can be from 3 to 5 hours.

The quantity of chlorine dioxide charged to the system is based on the amount of chlorine equivalent to the chlorine dioxide within the range from about 0.5 to about 3% Cl<sub>2</sub>, based on the weight of the dry pulp, and sometimes even more than 3 percent, up to about 5 percent. This treatment is also carried out in a manner to ensure a small excess, about 0.1 to 0.5% Cl<sub>2</sub>, at the end of the treatment.

The usual bleaching process for sulfate pulps includes six stages, in the order C E H D E D, the letters corresponding to the treatment stages set out above. An alkali extraction normally follows one or more stages of delignification, to remove solubilized lignins and other extractives. These stages can also be arranged in other combinations, for example,

C E C E H D E D  
C E H C H D E D  
C H E D E D  
C E D E D

Sulfite pulps can be bleached with shorter bleaching sequences, and illustrative sequences include

C E C E D  
C E H D  
C E D H  
C E H H  
C E H

It will be noted that in all of the sequences in common use for sulfate and sulfite pulps, the first treatment stage is invariably a chlorination stage, and the second treatment stage is almost invariably an alkali or extraction stage, to remove the lignins and other alkali-soluble extractives. In the single exception noted above, the hypochlorite stage serves as a substitute second chlorination stage, seeking to reduce the risk of cellulose decomposition in the first chlorination stage.

Anyhow as pointed out above also this hypochlorite stage comprises an alkali treatment immediately following the chlorination. An alkali extraction is interposed wherever more alkali-soluble extractives are to be removed.

The difficulty of control of the chlorination stage so as to prevent decomposition of the cellulose has drawn the attention of numerous workers in the pulp bleaching art, and many suggestions have been made. The most effective and least expensive alternatives, however, have involved the substitution of a hypochlorite or chlorine dioxide stage for a second chlorination stage, and a reduction in the severity of the first chlorination. Even in this variation, however, it is not possible to prevent decomposition of the cellulose altogether, particularly when the complementary stage is a hypochlorite treatment.

It has recently been proposed that the chlorination be carried out using a mixture of chlorine and chlorine dioxide. The amount of chlorine dioxide can be rather small, up to a major proportion. The chlorination is otherwise carried out in the usual way under the treatment conditions as set out in Table A above. However, the degree of amelioration obtained of the tendency to decompose the cellulose is not under these conditions sufficient to compensate for the considerable increase in the cost of the chlorination, due to the higher cost of chlorine dioxide as compared to chlorine. Moreover, the amelioration of the decomposition of the cellulose may also be accompanied by an incomplete delignification, as a result of which it becomes necessary to introduce another chlorination stage, or a hypochlorite or chlorine dioxide treatment stage, so as to complete the necessary delignification. In this event, there remains the possibility of decomposition of the cellulose during this complementary stage.

Ahlborg, U.S. Pat. No. 3,560,330, patented Feb. 2, 1971, proposes to delignify shives and specks which have not been sufficiently delignified in the first stage. The first delignification stage is a quite normal one, removing the bulk of lignin. In the second delignification stage, chlorine is added in a large excess, leaving as much as 2 to 10 grams of active chlorine per kilogram of pulp unreacted at the end of the treatment. The high concentration of active chlorine throughout the delignifying stage is claimed to be a prerequisite for an effective bleaching of the shives. The addition of chlorine dioxide in the second delignification stage is a secondary possibility, used to protect the cellulose in a way that has long been known. Such addition of a small amount of ClO<sub>2</sub> is a standard procedure in chlorination (see TAPPI Monograph No. 27, pp 135-136). This addition does not change the stage into something other than the normal chlorine stage, performed at a somewhat higher concentration of chlorine than usual. In the second stage, moreover, the temperature is held below 35° C., and preferably between 20° and 30° C.

In accordance with the instant invention, it has been determined that a second chlorination stage in which a mixture of chlorine and chlorine dioxide containing an

amount of chlorine dioxide within the range from about 10 to about 50 percent by weight of the mixture calculated as available chlorine is used at a pH within the range from about 1 to about 3.5 can be arranged to follow as a third or later stage a first chlorination stage, and a second alkali extraction stage, with good control of the decomposition of the cellulose pulp, as well as an at least substantially better delignification than in prior pulp treatment processes, and in many cases, a substantially complete delignification.

The objective of this invention is to remove lignin homogeneously throughout the body of cellulose pulp. An insufficient amount of delignifying agent is charged in the first delignification stage, leaving a substantial amount of lignin to be delignified in a subsequent stage. The charge in the second delignifying stage is sufficient to remove the remaining lignin, leaving no or only a small excess of available chlorine at the end of the treatment. The bleaching sequence includes a chlorine:chlorine dioxide stage, where the percentage of chlorine dioxide calculated as active chlorine is from about 10 to about 50 percent, preferably from 10 to 30 percent. Chlorine dioxide must be present. A pure chlorine stage would cause a severe degradation of the cellulose. The higher the temperature, the larger amount of chlorine dioxide that is needed. A high temperature, from 40° to 70° C. is used. Such a high temperature range has not earlier been possible in chlorination, due to cellulose degradation. The high temperature has been made possible by adding a sufficient amount of chlorine dioxide.

In the multistage pulp bleaching process of the invention, the first chlorination stage can be carried out with chlorine, with chlorine dioxide, or with a mixture of chlorine and chlorine dioxide either in the usual way, as shown in Table A, or preferably, under relatively mild conditions, so that delignification is incomplete. The cellulose pulp is then subjected to alkali treatment, and then in the third or some subsequent stage before the bleaching is complete, a continued delignification stage using a mixture of chlorine and chlorine dioxide in accordance with the invention.

The delignification stage of the invention is carried out under relatively severe conditions, unlike the preliminary chlorination stage, whether this stage is a normal chlorination, or a mild chlorination. In the delignification stage of the invention, the pH is within the range from about 1 to about 3.5. At a pH from 4 to 5 hypochlorous acid concentration reaches a maximum, and at a pH above 5, especially at from 6 to 7, the hypochlorous acid activity is at a maximum. This is undesirable, because of the degradation that results.

The pulp consistency is rather high, and is within the range from about 3 to about 15 percent. An ordinary chlorination stage without chlorine dioxide addition is carried out at 20° C. or lower. The temperature in the delignification stage of the invention is rather high, within the range from about 40° to about 70° C., and the treatment time is within the range from about 30 to about 300 minutes. These temperature and time conditions are not usually employed in a chlorination step, but correspond instead to the conditions of a hypochlorite or chlorine dioxide treatment.

In the delignification stage of the invention, the proportion of chlorine dioxide in the chlorine-chlorine dioxide mixture can be within the range from about 10 to about 50 percent chlorine dioxide, preferably within

the range from about 10 to about 30 percent chlorine dioxide. The amount is calculated in terms of the amount of available chlorine equivalent to the chlorine dioxide.

5 The chlorine is employed as chlorine liquid or chlorine gas, and is added to an aqueous suspension of the pulp in any conventional way. Chlorine dioxide is also added as such, or can be formed in situ. Usually, it is preferable to prepare chlorine dioxide as and when required, and then add it directly to the aqueous pulp mixture. Chlorine and chlorine dioxide should preferably be mixed thoroughly before the addition thereof into the aqueous pulp mixture.

10 The delignification stage of the invention offers several advantages over prior treatments, among them a lower cost for the chemicals required, and a very much smaller risk of decomposition of the cellulose. It is possible because of the benefits of the delignification stage of the invention to lower the cost for the chemicals required during bleaching, because of a reduction in the amounts of the chemicals, and rearrangement of the order of the various treatment stages of the bleaching process, with an unchanged or even improved quality of the pulp, in consequence.

15 In the process of the invention, the initial chlorination can be the usual chlorination described in Table A. Preferably, however, the chlorination stage is quite incomplete, and the chlorine charge rather small. Thus, the chlorine charge can be within the range from about 20 0.15 to about 0.25 percent chlorine per kappa number unit of the unbleached pulp, so that at the conclusion 30 of the chlorination a small excess, within the range from about 0.1 to about 0.5 percent chlorine, remains. Chlorine dioxide can be substituted in whole or in part 35 for chlorine, in amounts to supply an equivalent amount of chlorine, and an equivalent excess of chlorine at the conclusion of the process. Thus, mixtures of chlorine and chlorine dioxide can be used, with like effect. The treatment time can be rather small, as low as 40 twenty minutes, up to about two hours. Under these conditions, there is no noticeable decomposition of the cellulose.

45 The pulp consistency during this incomplete chlorination stage is within the usual range from about 1 to about 4%, and the temperature is also within the usual range from about 5° to about 25° C.

An alkali extraction stage is interposed following the chlorine-chlorine dioxide treatment of the invention to remove the alkali soluble lignin derivatives and other 50 alkali-soluble extractives formed in that stage. This alkali extraction can directly follow the  $\text{Cl}_2\text{-ClO}_2$  treatment, or be interposed at a later stage.

The alkali extraction can be under the usual conditions, as shown in Table A. However, lower alkali concentrations can be used, since a large proportion of alkali-soluble extractives will have been removed in the first alkali extraction. Thus, the amount of alkali can be from 0.5 to 1.5 percent, and at such amounts the pH will be from 8 to 12.5 at the end of the extraction, as 55 in the usual alkali extraction stage.

60 In the first alkali extraction, on the other hand, the application after an incomplete first chlorination implies a 15 to 25 percent saving in the amount of alkali, in this stage, in comparison to the application after a conventional chlorination. In the alkali extraction stage following the chlorine-chlorine dioxide treatment of the invention, the pulp consistency is within the usual

range from about 4 to about 18 percent, the temperature within the usual range from about 25° to about 30° C., up to about 130° C. in a hot alkali refining stage, and the treatment time can range from several minutes to about 5 hours.

Following the chlorination and alkali extraction stages, the pulp is then subjected to the delignification stage in accordance with the invention. The pulp at this point may well be less completely delignified than after conventional chlorination and alkali extraction processes, but nonetheless, at the conclusion of the delignification stage of the invention, the resulting pulp is more delignified and has a better quality. This means that the final bleaching of the delignified pulp can be performed with less chemical consumption and results in better quality of the final bleached pulp. Quality of the final bleached pulp is evaluated by the usual criteria: (1) brightness, percent SCAN before and after aging at elevated temperatures, (2) viscosity (which is determined for an aqueous copper ethylene diamine solution of the pulp according to SCAN C15:62, and which is a measurement of the mean polymerization degree of the cellulose, i.e., the chain length of the cel-

lulose molecules, and (3) the extinction at 205 nm, i.e., ultraviolet light (which is determined for a solution of the pulp in phosphoric acid containing 5 mg. of pulp per ml. and is a measurement of the quantity of lignin remaining in the pulp). The higher the viscosity, the greater the strength of the pulp, and the lower the extinction, the greater the extent of delignification.

The following Examples represent preferred embodiments of the invention.

### EXAMPLE 1

15 An unbleached cellulose pulp prepared from pine wood by the sulfate process, having a kappa number of 31 (the kappa number is a measurement of the lignin content of the pulp, and thus of its consumption of bleaching chemicals. The determination of kappa number is according to the standard in SCAN-C 1:59) was chlorinated and treated with alkali as the first two 20 stages of the bleaching process. The pulp was then divided into four batches, and the bleaching was continued in a series of steps. The conditions are outlined in Table I.

TABLE I

| Stage Treatment                                          | BATCH NUMBER            |                               |                               |                               |
|----------------------------------------------------------|-------------------------|-------------------------------|-------------------------------|-------------------------------|
|                                                          | 1                       | 2                             | 3                             | 4                             |
| <b>(1) Chlorination</b>                                  |                         |                               |                               |                               |
| Pulp consistency                                         |                         | 3.5%                          |                               |                               |
| Temperature                                              |                         | 20°C.                         |                               |                               |
| Chlorine charge <sup>2</sup>                             |                         | 6.8%                          |                               |                               |
| Treatment time                                           |                         | 1 hour                        |                               |                               |
| Chlorine residue at end of treatment                     |                         | 0.15% <sup>2</sup>            |                               |                               |
| <b>(2) Alkali Extraction</b>                             |                         |                               |                               |                               |
| Pulp consistency                                         |                         | 8%                            |                               |                               |
| Temperature                                              |                         | 50°C.                         |                               |                               |
| NaOH charge                                              |                         | 3% <sup>2</sup>               |                               |                               |
| Treatment time                                           |                         | 2 hours                       |                               |                               |
| pH at end of treatment                                   |                         | 11.6                          |                               |                               |
| <b>(3)</b>                                               |                         |                               |                               |                               |
|                                                          | HOCl                    | CHLORINE + ClO <sub>2</sub>   |                               |                               |
| Pulp consistency                                         | 8%                      | 6%                            | 6%                            | 6%                            |
| Temperature °C.                                          | 45°                     | 40°                           | 40°                           | 60°                           |
|                                                          | NaOCl <sup>1</sup>      | Cl <sub>2</sub>               | Cl <sub>2</sub>               | Cl <sub>2</sub>               |
| Charge <sup>2</sup>                                      | 1.7%                    | 1.08%                         | 0.775%                        | 1.08%                         |
|                                                          | NaOH                    | ClO <sub>2</sub> <sup>1</sup> | ClO <sub>2</sub> <sup>1</sup> | ClO <sub>2</sub> <sup>1</sup> |
| Charge <sup>2</sup>                                      | 0.68%                   | 0.47                          | 0.775                         | 0.47                          |
| Treatment time (hours)                                   | 2                       | 3                             | 3                             | 3                             |
| Chlorine excess at end of treatment                      | 0.2% 0.06% <sup>2</sup> | 0.02 <sup>2</sup>             | 0.01% <sup>2</sup>            |                               |
| pH at end of treatment                                   | 10.7                    | 2.1                           | 2.15                          | 2.1                           |
| <b>(4) Alkali Extraction</b>                             |                         |                               |                               |                               |
| Pulp consistency                                         | None                    |                               |                               |                               |
| Temperature                                              |                         | 50°C.                         |                               |                               |
| NaOH charge                                              |                         | 1% <sup>2</sup>               |                               |                               |
| Treatment time (hours)                                   |                         | 2                             |                               |                               |
| pH at end of treatment                                   |                         | 11.5                          |                               |                               |
| <b>(5) Chlorine Dioxide</b>                              |                         |                               |                               |                               |
| Pulp consistency                                         |                         | 6%                            |                               |                               |
| Temperature                                              |                         | 70°C.                         |                               |                               |
| ClO <sub>2</sub> charge (as equivalent Cl <sub>2</sub> ) |                         | 1% <sup>2</sup>               |                               |                               |
| Treatment time (hours)                                   |                         | 3                             |                               |                               |
| Surplus chlorinating equivalent at end of treatment      |                         | 0.05 to 0.20% <sup>2</sup>    |                               |                               |

Table I—Continued

| Stage Treatment                                            | BATCH NUMBER |                       |                   |      |
|------------------------------------------------------------|--------------|-----------------------|-------------------|------|
|                                                            | 1            | 2                     | 3                 | 4    |
| <b>(6) Alkali Extraction</b>                               |              |                       |                   |      |
| Pulp consistency                                           |              |                       | 8%                |      |
| Temperature                                                |              |                       | 50°C.             |      |
| NaOH charge                                                |              |                       | 0.7% <sup>2</sup> |      |
| Treatment time (hours)                                     |              |                       | 2                 |      |
| pH at end of treatment                                     |              |                       | 11.2-11.3         |      |
| <b>(7) Chlorine Dioxide</b>                                |              |                       |                   |      |
| Pulp consistency                                           |              | 6%                    |                   |      |
| Temperature                                                |              | 85°C.                 |                   |      |
| ClO <sub>2</sub> charge (as equivalent Cl <sub>2</sub> )   |              | 0.9% <sup>2</sup>     |                   |      |
| Treatment time                                             |              | 5 hours               |                   |      |
| Surplus chlorine equivalent at end of treatment (%)        |              | 0.2-0.3% <sup>2</sup> |                   |      |
| <b>PROPERTIES OF BLEACHED PULPS</b>                        |              |                       |                   |      |
| Brightness, % SCAN                                         | 93.6         | 93.7                  | 93.7              | 93.6 |
| Brightness after ageing 16 hours at 180°C., 80% rh         | 86.8         | 87.7                  | 87.1              | 83.2 |
| Brightness after ageing 16 hours at 120°C., dry atmosphere | 87.7         | 88.3                  | 88.0              | 88.5 |
| Viscosity, cp Tappi                                        | 44           | 55                    | 55                | 59   |
| Extinction at -205 nm, cm <sup>1</sup>                     | 0.35         | 0.31                  | 0.30              | 0.36 |

<sup>1</sup> based on Cl<sub>2</sub> equivalent<sup>2</sup> dry pulp weight

Batch 1 served as a control in which a conventional hypochlorite treatment was used as stage (3) instead of the chlorine-chlorine dioxide treatment in accordance with the invention, which was used for batches 2 to 4. It is apparent from the properties of the finished pulp that pulps of equivalent or improved brightness were obtained using the chlorine-chlorine dioxide treatment of the invention. These pulps also had a distinctly higher viscosity, and a lower extinction. The viscosity for a sulfate pulp up to viscosities up to approximately 60 cp Tappi shows a direct correlation between the strength of paper produced from the pulp, and the magnitude of viscosity. At levels above 60 cp Tappi, increases in the viscosity may improve strength but not to the same extent.

Data show that replacement of the hypochlorite treatment stage with the delignification stage of the invention gives an increase in the potential strength properties of the pulp, and an improved delignification. Moreover, there is a marked reduction in the chemical costs for bleaching in the case of batches 2 to 4, as compared to batch 1.

**EXAMPLE 2**

Using the same starting cellulose pulp as in Example 1, a bleaching operation was carried out in accordance with the stages outlined in Table I, except that in the first chlorination stage, 5 percent of the chlorine

charge was replaced by an equivalent quantity of chlorine dioxide. The results obtained were similar to those shown in Table I, with the exception that the viscosities were higher:

**TABLE II**

| Batch No. | 1                   | 2  | 3  | 4  |
|-----------|---------------------|----|----|----|
|           | Viscosity, cp Tappi | 64 | 87 | 76 |

Because of the use of the chlorine dioxide in substitution for chlorine, the cost for the chemicals was somewhat higher than the cost of the process outlined in Table I.

**EXAMPLE 3**

This Example illustrates the improvement obtained when combining the chlorine-chlorine-dioxide delignification stage of the invention with a milder chlorination first stage, with incomplete delignification. An unbleached pulp derived from pine wood by the sulfate process and having a kappa number of 31 was used. This was divided into six batches, which were bleached in accordance with the stages outlined in Table III. Batches 1, 2 and 3 were controls, and batches 4 to 6 illustrate the use of the chlorine-chlorine dioxide delignification of the invention, as stage (3), in replacement of the hypochlorite stage (3) used for batches 1 to 3.

**TABLE III**

| Stage Treatment                      | BATCH NUMBER |       |       |   |   |   |
|--------------------------------------|--------------|-------|-------|---|---|---|
|                                      | 1            | 2     | 3     | 4 | 5 | 6 |
| <b>(1) Chlorination</b>              |              |       |       |   |   |   |
| Pulp consistency                     | 3.5%         | 3.5%  | 3.5%  |   |   |   |
| Temperature                          | 20°C.        | 20°C. | 20°C. |   |   |   |
| Cl <sub>2</sub> charge <sup>2</sup>  | 6.8%         | 6.46% | 5.25% |   |   |   |
| ClO <sub>2</sub> charge <sup>2</sup> | —            | 0.34% | —     |   |   |   |
| Time (hours)                         | 1            | 1     | 1     |   |   |   |
| Cl <sub>2</sub> excess               | 0.2%         | 0.2%  | 0.1%  |   |   |   |

TABLE III - Continued

| Stage Treatment                                               | BATCH NUMBER |      |      |                              |                |                                  |
|---------------------------------------------------------------|--------------|------|------|------------------------------|----------------|----------------------------------|
|                                                               | 1            | 2    | 3    | 4                            | 5              | 6                                |
| <b>(2) Alkali Extraction</b>                                  |              |      |      |                              |                |                                  |
| Pulp consistency                                              | 8%           |      |      |                              |                | 8%                               |
| Temperature                                                   | 50°C.        |      |      |                              |                | 50°C.                            |
| NaOH charge <sup>2</sup>                                      | 3%           |      |      |                              |                | 2.3%                             |
| Time (hours)                                                  | 2            |      |      |                              |                | 10.9-11.4                        |
| pH at end of treatment                                        | 10.9-11.4    |      |      |                              |                | 10.9-11.4                        |
| <b>(3)</b>                                                    |              |      |      |                              |                |                                  |
|                                                               | Hypochlorite |      |      | $\text{Cl}_2 + \text{ClO}_2$ |                |                                  |
| Pulp consistency                                              | 8%           | 8%   | 8%   | 6%                           | 6%             | 6%                               |
| Temperature °C.                                               | 40°          | 40°  | 40°  | 40°                          | 40°            | 40°                              |
| NaOCl <sup>1</sup>                                            |              |      |      | $\text{Cl}_2$                | $\text{Cl}_2$  | $\text{Cl}_2$                    |
| Charge <sup>2</sup>                                           | 1.08         | 1.08 | 2.32 | 1.94                         | 1.73           | 1.51                             |
| NaOH                                                          |              |      | NaOH | $\text{ClO}_2$               | $\text{ClO}_2$ | $\text{ClO}_2$                   |
| Charge <sup>2</sup>                                           | 0.43         | 0.43 | 0.93 | 0.22                         | 0.43           | 0.65                             |
| Time (hours)                                                  | 2            | 2    | 2    | 3                            | 3              | 3                                |
| pH at end of treatment                                        | 10.6         | 10.9 | 10.9 | 1.65                         | 1.7            | 1.85                             |
| $\text{Cl}_2$ equivalent <sup>2</sup> at end of treatment (%) | 0.05         | 1    | 0.10 | 0.02                         | 0.02           | 0.02                             |
| <b>(4) Alkali Extraction</b>                                  |              |      |      |                              |                |                                  |
| Pulp consistency                                              |              |      | None |                              |                | 8%                               |
| Temperature                                                   |              |      |      |                              |                | 50°C.                            |
| NaOH charge <sup>2</sup>                                      |              |      |      |                              |                | 1%                               |
| Time (hours)                                                  |              |      |      |                              |                | 2                                |
| pH at end of treatment                                        |              |      |      |                              |                | 11-11.2                          |
| <b>(5) Chlorine Dioxide</b>                                   |              |      |      |                              |                |                                  |
| Pulp consistency                                              | 6%           |      |      |                              |                | 6%                               |
| Temperature                                                   |              |      |      |                              |                | 70°C.                            |
| $\text{ClO}_2$ charge (as equivalent $\text{Cl}_2$ )          |              |      |      |                              |                | 1% of dry pulp weight            |
| Time (hours)                                                  |              |      |      |                              |                | 3                                |
| Surplus chlorine equivalent at end of treatment               |              |      |      |                              |                | 0.05 to 0.20% of dry pulp weight |
| <b>(6) Alkali Extraction</b>                                  |              |      |      |                              |                |                                  |
| Pulp consistency                                              |              |      |      |                              |                | 8%                               |
| Temperature                                                   |              |      |      |                              |                | 50°C.                            |
| NaOH charge                                                   |              |      |      |                              |                | 0.7% of dry pulp weight          |
| Time (hours)                                                  |              |      |      |                              |                | 2                                |
| pH at end of treatment                                        |              |      |      |                              |                | 11.2-11.3                        |
| <b>(7) Chlorine Dioxide</b>                                   |              |      |      |                              |                |                                  |
| Pulp consistency                                              |              |      |      |                              |                | 6%                               |
| Temperature                                                   |              |      |      |                              |                | 85°C.                            |
| $\text{ClO}_2$ charge (as equivalent $\text{Cl}_2$ )          |              |      |      |                              |                | 0.9% of dry pulp weight          |
| Time (hours)                                                  |              |      |      |                              |                | 5                                |
| Surplus chlorine equivalent at end of treatment               |              |      |      |                              |                | 0.2-0.3% dry pulp weight         |
| <b>Bleached Pulp Properties</b>                               |              |      |      |                              |                |                                  |
| Brightness, % SCAN                                            | 91.9         | 91.7 | 93.0 | 92.9                         | 92.4           | 92.2                             |
| Ditto after ageing for 16 hrs/80°C., 80% rh                   | 85.2         | 84.9 | 84.5 | 85.4                         | 85.3           | 84.8                             |
| Ditto after ageing 16 hrs/120°C., dry atmosphere              | 85.4         | 85.1 | 85.1 | 86.9                         | 86.2           | 85.6                             |
| Viscosity, cP Tappi                                           | 56           | 89   | 68   | 86                           | 90             | 93                               |
| Extinction at 205 nm, $\text{cm}^{-1}$                        | 0.38         | 0.40 | 0.53 | 0.36                         | 0.36           | 0.35                             |

<sup>1</sup> based on  $\text{Cl}_2$  equivalent<sup>2</sup> dry pulp weight

It is evident from the data that the cost for the chemicals in the treatment of batches 4 to 6 was reduced, and in spite of this an improved brightness was obtained, as

compared to batches 1 to 3. Batches 4, 5 and 6 gave as high a viscosity as in the case of batch 2, in which the bleaching was conducted with the addition of chlorine

dioxide in the chlorination stage. Moreover, the final delignification is more complete, as indicated by the extinction values for batches 4 to 6.

#### EXAMPLE 4

This Example shows that if a delignification stage in accordance with the invention is employed, delignification prior to final bleaching can be carried further than in a conventional bleaching process, without the

viscosity of the pulp being impaired. This makes it possible to reduce the final bleaching process to one chlorine dioxide stage instead of two chlorine dioxide stages, with an intermediate alkali stage.

In the experiments which are described here, an unbleached cellulose pulp derived from pine wood by the sulfate process was used, having a kappa number of 34.7. This was divided into four batches, and the batches were treated as outlined in Table IV:

TABLE IV

| Stage Treatment                                                 | BATCH NUMBER                           |                    |                                        |                                        |
|-----------------------------------------------------------------|----------------------------------------|--------------------|----------------------------------------|----------------------------------------|
|                                                                 | 1                                      | 2                  | 3                                      | 4                                      |
| <b>(1) Chlorination</b>                                         |                                        |                    |                                        |                                        |
| Pulp consistency                                                | 3.5%                                   | 3.5%               | 3.5%                                   | 3.5%                                   |
| Temperature                                                     | 20°C.                                  | 20°C.              | 20°C.                                  | 20°C.                                  |
| % Cl <sub>2</sub> <sup>2</sup>                                  | 7.22                                   | 7.22               | 5.6                                    | 5.6                                    |
| % ClO <sub>2</sub> <sup>12</sup>                                | 0.38                                   | 0.38               | 0.30                                   | 0.30                                   |
| Time                                                            | 1 hour                                 | 1 hour             | 20 min.                                | 20 min.                                |
| Cl <sub>2</sub> excess at end of treatment                      | 0.3                                    | 0.3                | 0.1                                    | 0.1                                    |
| <b>(2) Alkali Extraction</b>                                    |                                        |                    |                                        |                                        |
| Pulp consistency                                                |                                        |                    | 8%                                     |                                        |
| Temperature                                                     |                                        |                    | 50°C.                                  |                                        |
| % NaOH <sup>2</sup>                                             |                                        |                    | 2.8%                                   |                                        |
| Time                                                            |                                        |                    | 2 hours                                |                                        |
| pH at end of treatment                                          |                                        |                    | 11.1-11.5                              |                                        |
| <b>(3)</b>                                                      |                                        |                    |                                        |                                        |
|                                                                 | Hypochlorite                           |                    | Cl <sub>2</sub> -ClO <sub>2</sub>      |                                        |
| Pulp consistency                                                | 8%<br>40°C.                            | 8%<br>40°C.        | 6%<br>50°C.                            | 6%<br>50°C.                            |
| Temperature                                                     | NaOCl <sup>1</sup>                     | NaOCl <sup>1</sup> | Cl <sub>2</sub>                        | Cl <sub>2</sub>                        |
| Charge <sup>2</sup>                                             | 1.9%<br>NaOH                           | 1.9%<br>NaOH       | 2.38%<br>ClO <sub>2</sub> <sup>1</sup> | 2.38%<br>ClO <sub>2</sub> <sup>1</sup> |
| Charge <sup>2</sup>                                             | 0.73%<br>2                             | 0.73%<br>2         | 0.42%<br>3                             | 0.42%<br>3                             |
| Time (hours)                                                    | 0.43                                   | 0.43               | 0.23%                                  | 0.23%                                  |
| Cl <sub>2</sub> excess at end of treatment                      | 11.0                                   | 11.0               | 1.7                                    | 1.7                                    |
| pH at end of treatment                                          |                                        |                    |                                        |                                        |
| <b>(4) Alkali Extraction</b>                                    |                                        |                    |                                        |                                        |
| Pulp consistency                                                | None                                   |                    | 8%<br>50°C.                            | 8%<br>50°C.                            |
| Temperature                                                     |                                        |                    | 1%                                     | 1%                                     |
| % NaOH <sup>2</sup>                                             |                                        |                    | 2 Hours                                | 2 Hours                                |
| Time                                                            |                                        |                    | 10.95                                  | 10.95                                  |
| pH at end of treatment                                          |                                        |                    |                                        |                                        |
| <b>(5) ClO<sub>2</sub></b>                                      |                                        |                    |                                        |                                        |
| Pulp consistency                                                | 8%<br>70                               | None               | 8%<br>70                               | 8%<br>85                               |
| Temperature°C.                                                  | ClO <sub>2</sub> <sup>12</sup><br>1.3% |                    | 2.0%                                   | 1.3%<br>2.0%                           |
| Time                                                            | 3 hours<br>0.6                         | 5 hours<br>0.07    | 3 hours<br>0.20                        | 5 hours<br>0.16                        |
| Cl <sub>2</sub> equivalent <sup>2</sup> at end of treatment (%) |                                        |                    |                                        |                                        |
| <b>(6) Alkali Extraction</b>                                    |                                        |                    |                                        |                                        |
| Pulp consistency                                                | 8%<br>50°C.                            | None               | 8%<br>50°C.                            | None                                   |
| Temperature                                                     | 0.7%                                   |                    | 0.7%                                   |                                        |
| % NaOH <sup>2</sup>                                             | 2 hours                                |                    | 2 hours                                |                                        |
| Time                                                            |                                        |                    |                                        |                                        |
| pH at end of treatment                                          | 11.1-11.2                              |                    | 11.1-11.2                              |                                        |

TABLE IV - Continued

| Stage Treatment                                                 | BATCH NUMBER |       |           |       |
|-----------------------------------------------------------------|--------------|-------|-----------|-------|
|                                                                 | 1            | 2     | 3         | 4     |
| <b>(7) ClO<sub>2</sub></b>                                      |              |       |           |       |
| Pulp consistency                                                | 6%           |       |           |       |
| Temperature                                                     | 85°C.        | None  | 6%        | None  |
| ClO <sub>2</sub> <sup>1</sup>                                   | 0.9%         |       | 0.9%      |       |
| Time                                                            | 5 hours      |       | 5 hours   |       |
| Cl <sub>2</sub> equivalent <sup>2</sup> at end of treatment (%) | 0.13-0.14    |       | 0.13-0.14 |       |
| <b>Properties of Bleached Pulp</b>                              |              |       |           |       |
| Brightness according to SCAN, %                                 | 93.3         | 90.6  | 94.1      | 92.1  |
| Brightness after ageing for 16 hours at 80°C., 80% rh           | 86.3         | 83.5  | 86.9      | 85.4  |
| Brightness after ageing for 16 hours at 120°C., dry atmosphere  | 87.3         | 83.4  | 89.0      | 85.2  |
| Viscosity according to Tappi cP                                 | 61           | 50    | 65        | 61    |
| Extinction at 205 nm, cm <sup>-1</sup>                          | 0.361        | 0.481 | 0.293     | 0.364 |

<sup>1</sup> based on Cl<sub>2</sub> equivalent<sup>2</sup> dry pulp weight

It is apparent from the data that batch 2, delignified according to the conventional procedure using hypochlorite, and batch 4, delignified in accordance with the present invention, which were finally bleached using only one chlorine dioxide stage, showed a lower degree of brightness than corresponding pulps finally bleached with two chlorine dioxide stages, batches 1 and 3, respectively. The brightness of the pulp batch 4 delignified in accordance with the invention lay at an acceptable level, and the viscosity is as high as that of batch 1, which was bleached with two chlorine dioxide stages in the final bleaching stage, but with conventional delignification including a hypochlorite stage.

Delignification according to the invention followed by final bleaching, using only one chlorine dioxide stage, can be considered as a modification of the generally used sequence C E D E D. The invention thus provides a reduced cost of chemicals, and gives good pulp quality with regard to brightness and mechanical strength. Also, when using the process of the invention, it is possible to carry the delignification further with chlorine than is otherwise possible, which in turn makes it possible to carry the final bleaching stage to the desired degree of brightness with only one intensive chlorine dioxide treatment stage.

Having regard to the foregoing disclosure, the following is claimed as the inventive and patentable embodiments thereof:

1. A multistage pulp bleaching and delignification process comprising in a first chlorination and delignification stage chlorinating cellulose pulp with chlorine, with chlorine dioxide, or with a mixture of chlorine and chlorine dioxide under relatively mild conditions, so that delignification is incomplete; in an alkali treatment stage alkali-treating the chlorinated pulp; and then, as a third or subsequent stage, before the bleaching is complete, in a second chlorination and delignification stage, chlorinating the alkali treated pulp with a mixture of chlorine and chlorine dioxide comprising from about 10 percent to about 50 percent chlorine dioxide

calculated as available chlorine at a pH within the range from about 1 to about 3.5 and at a pulp consistency within the range from about 3 to about 15 percent, and a temperature within the range from about 40° to about 70° C., for a time within the range from about 30 to about 300 minutes.

2. A process in accordance with claim 1, which comprises chlorinating the pulp in the first chlorination and delignification stage with chlorine.

3. A process in accordance with claim 1, which comprises alkali treating the chlorinated pulp subsequent to the second chlorination and delignification stage.

4. A process in accordance with claim 1, which comprises alkali treating the delignified pulp and then treating the alkali treated delignified pulp with a member selected from group consisting of hypochlorite and chlorine dioxide.

5. A process in accordance with claim 1, in which the first chlorination and delignification is effected at a pulp consistency within the range from about 1 to about 4 percent, a temperature from about 5° to about 25° C. for from about 1/3 to about 2 hours, with sufficient chlorine, supplied as chlorine, chlorine dioxide, or both, to provide from about 0.1 to about 0.5 percent excess chlorine at the end of the chlorination.

6. A process in accordance with claim 1, in which the alkali treatment is effected at a pulp consistency within the range from about 4 to about 18 percent at a temperature from about 25° to about 130° C. for a period of time up to about 5 hours, and with sufficient alkali to afford a pH from about 8 to about 12.5 at the end of the alkali treatment.

7. A process in accordance with claim 1, in which the proportion of chlorine dioxide in the chlorine-chlorine dioxide mixture in the second chlorination and delignification stage is within the range from about 10 to about 30 percent chlorine dioxide, calculated as the amount of chlorine equivalent to the chlorine dioxide.

\* \* \* \* \*

UNITED STATES PATENT OFFICE  
CERTIFICATE OF CORRECTION

Patent No. 3,802,958 Dated April 9, 1974

Inventor(s) Ingemar Liss-Albin Croon et al.

It is certified that error appears in the above-identified patent and that said Letters Patent are hereby corrected as shown below:

Page 1, [ 75] line 2 : after "Salgvagen" insert --Domsjoverken--

line 3 : after "Strandvagen" insert --Hallstavik--

Column 4, line 43 : after "delignification" please insert a period  
--.--.

Column 7, line 6 : "FOllowing" should be -- Following--

UNITED STATES PATENT OFFICE  
CERTIFICATE OF CORRECTION

Patent No. 3,802,958Dated April 9, 1974Inventor(s) Ingemar Liss -Albin Croon et al.

It is certified that error appears in the above-identified patent and that said Letters Patent are hereby corrected as shown below:

Column 8, Table I, heading (3) Batches 1, 2, 3 and 4

should be

| (3)                                 | HOCl  | CHLORINE + ClO <sub>2</sub>   |                               |                               |
|-------------------------------------|-------|-------------------------------|-------------------------------|-------------------------------|
|                                     |       | 6%                            | 6%                            | 6%                            |
| Pulp consistency                    | 8%    |                               |                               |                               |
| Temperature °C.                     | 45°   | 40°                           | 40°                           | 60°                           |
| Charge <sup>2</sup>                 |       |                               |                               |                               |
| NaOCl <sup>1</sup>                  |       | Cl <sub>2</sub>               | Cl <sub>2</sub>               | Cl <sub>2</sub>               |
| 1.7%                                |       | 1.08%                         | 0.775%                        | 1.08%                         |
| NaOH                                |       | ClO <sub>2</sub> <sup>1</sup> | ClO <sub>2</sub> <sup>1</sup> | ClO <sub>2</sub> <sup>1</sup> |
| Charge <sup>2</sup>                 | 0.68% | 0.47                          | 0.775                         | 0.47                          |
| Treatment time (hours)              | 2     | 3                             | 3                             | 3                             |
| Chlorine excess at end of treatment | 0.2%  | 0.06% <sup>2</sup>            | 0.02% <sup>2</sup>            | 0.01% <sup>2</sup>            |
| pH at end of treatment              | 10.7  | 2.1                           | 2.15                          | 2.1                           |

UNITED STATES PATENT OFFICE  
CERTIFICATE OF CORRECTION

Patent No. 3,802,958 Dated April 9, 1974

Inventor(s) Ingemar Liss - Albin Croon et al.

It is certified that error appears in the above-identified patent and that said Letters Patent are hereby corrected as shown below:

Column 8, Table I, heading 4, Batch 3

should be

| <u>(4) Alkali Extraction</u> |      |  |       |
|------------------------------|------|--|-------|
| Pulp consistency             | None |  | 8%    |
| Temperature                  |      |  | 50°C. |
| NaOH charge                  |      |  | 1%    |
| Treatment time (hours)       |      |  | 2     |
| pH at end of treatment       |      |  | 11.5  |

**UNITED STATES PATENT OFFICE**  
**CERTIFICATE OF CORRECTION**

Patent No. 3,802,958Dated April 9, 1974Inventor(s) Ingemar Liss-Albin Croon et al

It is certified that error appears in the above-identified patent and that said Letters Patent are hereby corrected as shown below:

Column 14, Table IV, heading (5) Batch 2

should be

| (5) <u>ClO<sub>2</sub></u>                         |         |         |         |         |
|----------------------------------------------------|---------|---------|---------|---------|
| Pulp consistency                                   | 8%      | 8%      | 8%      | 8%      |
| Temperature °C.                                    | 70      | 85      | 70      | 85      |
| ClO <sub>2</sub> <sup>1</sup> / <sub>2</sub>       | 1.3%    | 2.0%    | 1.3%    | 2.0%    |
| Time                                               | 3 hours | 5 hours | 3 hours | 5 hours |
| Cl <sub>2</sub> equivalent at end of treatment (%) | 0.6     | 0.07    | 0.20    | 0.16    |

Column 15, line 40 : "sequency" should be --sequence--

Signed and Sealed this

thirtieth Day of March 1976

[SEAL]

Attest:

**RUTH C. MASON**  
*Attesting Officer*

**C. MARSHALL DANN**  
*Commissioner of Patents and Trademarks*